# EUROPEAN PATENT SPECIFICATION

(11) **EP 2 754 511 B1**
(45) Date of publication and mention of the grant of the patent: **08.08.2018**
(21) Application number: 14150765.7
(22) Date of filing: 10.01.2014
(51) Int. Cl.: B21F 27/10, B21C 1/02, C21D 7/10

(54) **Method for manufacturing a steel wire mesh**
Methode zur Herstellung einer Gittermatte
Méthode pour la fabrication d'un mât en treillis

(30) Priority: 11.01.2013 FI 20135036
(43) Date of publication of application: 16.07.2014
(73) Proprietor: Tammet Oy, 10600 Tammisaari (FI)
(72) Inventor: Heikkilä, Tarmo, 36600 Pälkäne (FI)
(74) Representative: Berggren Oy, Turku

(56) References cited:
- EP-A1- 0 780 174
- WO-A1-00/51760
- AU-B2- 2002 300 805

## Description

### Field of the invention

The invention relates to a method for manufacturing a steel wire mesh according to the preamble of the enclosed independent claim.

### Background of the invention

A mesh manufactured from steel wire, a so-called steel wire mesh for mining applications, is attached to the walls of mine tunnels and respective structures to reinforce the tunnel structure and to prevent the falling of loose rocks. The used steel wire mesh for mining applications should conform to the walls of the tunnel, so the steel wire mesh for mining applications should be manufactured from a wire having an appropriate ductility. However, there are certain strength requirements for the steel wire to be used in the manufacture of the mesh depending on the purpose of use, so that the mesh structure manufactured from it will last in the purpose of use. The steel wire mesh for mining applications manufactured should, however, be relatively easy to shape, so that it can be shaped by mechanical pressing to conform to the walls of the tunnel.

Typically, the steel wire meshes for mining applications are manufactured from wire rod, so that the wire rod made of steel having a specific diameter is first guided to a cold forming stage, in which the diameter of the wire rod is substantially decreased to a desired wire diameter to be used in the final mesh structure. The diameter of the wire rod is typically decreased by 8-30%. Cold forming can either be carried out by rolling or cold extension. Cold forming requires one or several successive rolls or drawing stones having a different aperture, since the diameter of the rod can only be decreased a certain amount at once. Cold forming reinforces the wire, so that after the cold forming the steel wire has to be heat treated in order to achieve the desired softness and shapability, so that the wire can be used in the manufacture of steel wire mesh for mining applications. The heat treatment consumes remarkable amounts of energy and increases thus the production costs of the mesh manufactured from the steel wire. After the heat treatment the annealed steel wire is straightened and cut into the desired length, after which a desired mesh structure is prepared from the wire by welding.

Document WO 00/51760, which forms the basis for the preamble of claim 1, discloses a method and installation for producing grid mats comprised of rods which are welded to one another at crossing points. Rods are continuously drawn from each wire supply and stretched, subsequently temper rolled and cut into lengths.

Document AU 2002300805 discloses a method, which involves cold working a wire uch that the cross-sectional area of the wire is reduced by 5% to 15% and the wire retains a ductility greater than 5%.

### Object and description of the invention

The object of the present invention is to provide a method for manufacturing a steel wire mesh, preferably a steel wire mesh for mining applications, from a steel wire rod, which method is simpler and thus more cost-effective than the conventional production method.

To achieve this object, the method according to the invention is characterised in what is presented in the characterising part of the independent claim.

The other, dependent claims present some preferred embodiments of the invention.

A typical method of the invention for manufacturing a steel wire mesh, preferably a steel wire mesh for mining applications, from steel wire rod is described in claim 1.

A typical system for manufacturing a steel wire mesh, preferably a steel wire mesh for mining applications, from steel wire rod, comprises at least
- means for guiding steel wire rod into a further processing stage,
- means for further processing the steel wire rod,
- means for straightening the processed steel wire rod and cutting it into parts having a desired length, and
- means for welding the mesh from the steel wire parts.

The system is free from heat treatment means and the further processing means of the steel wire rod are arranged so that the average diameter of the steel wire rod does not substantially change in the further processing stage.

In a method according to the invention the average diameter the steel wire rod does not substantially change, i.e. the average diameter of the wire rod remains substantially the same.

Typically, the steel wire mesh, which is manufactured by the method of the invention, is used in the walls of mine tunnels and corresponding structures to reinforce the tunnel structure and to prevent the falling of loose rocks. Typically, the mesh manufactured by the method according to the invention is thus used as a so-called steel wire mesh for mining applications. The steel wire mesh for mining applications is typically a planar and ductile steel mesh, which can be attached to the wall of the mine tunnel or corresponding structure, and after attaching the mesh the tunnel walls can be shotcreted.

It has now been surprisingly found that the steel wire mesh for mining applications or corresponding mesh structure having a sufficient strength and shapability can be easily and simply manufactured from the steel wire rod having a specific diameter, which steel wire rod meets the desired strength and shapability requirements, without a separate heat treatment stage. The steel wire rod which used as a raw material in the method according to the invention for manufacturing a steel wire mesh is only guided through a further processing stage and straightening stage before forming the actual mesh structure by welding. In other words, in the method according to the invention the steel wire rod is typically guided straight from the further processing stage to the straightening stage, optionally through intermediate coiling, but without any intermediate stages, which would affect the strength properties of the wire. Thus, the manufacturing method according to the invention, which method is free from the heat treatment stages of the steel wire rod, is remarkably simpler and more cost-effective than the manufacturing method according to the prior art.

In the method according to the invention the further processing stage is only a so-called calibration stretch, the meaning of which is not to substantially change the average diameter of the wire rod, but the average diameter of the steel wire rod is mainly the same before the further processing stage and after it. The average diameter of the steel wire rod means the mathematical mean value of the diameters measured at several locations of the wire. The further processing is however performed, so that roll scale and other possible slag and impurities, which hinder the welding of the mesh from the steel wire, can be removed from the surface of the steel wire rod to be used as a material of the mesh. Simultaneously, the diameter of the wire is formed more circular, since the cross-section of the unprocessed steel wire rod is typically not entirely circular, but it may be oval-shaped or otherwise deformed.

According to the invention the change of the average diameter of the wire rod is 0.01-0.75%.

In one embodiment method according to the invention the further processing, i.e. the calibration stretch, is performed by guiding the steel wire rod through at least one drawing stone, drawing stone aperture being a diameter which is substantially the same as the average diameter of the steel wire rod. In a preferred embodiment the steel wire rod is guided through only one drawing stone, wherein the process is as simple as possible. Alternatively, the further processing can be performed in a method according to the invention by directing the steel wire rod through one or more rolling units, so that the average diameter of the steel wire rod does not substantially change. In one preferred embodiment the steel wire rod is guided in the further processing stage through only one rolling unit so that the average diameter of the wire rod does not substantially change.

Since the calibration stretch stage is only meant to remove roll scale from the surface of the steel wire rod to be used as a raw material for the steel wire mesh, the production speed of this stage can be kept high. In an embodiment of the invention the production speed, which here means the propagation speed of the steel wire rod in the further processing stage, is substantially the same as the maximum speed of a wire coiling unit used in the further processing. The production rate is for example about 10 m/s. The production rate is thus not affected by directing the steel wire rod through the further processing means, such as drawing stone or twin rolls.

The steel wire rod used in the method according to the invention is a wire manufactured from steel by hot rolling, the diameter of which wire is typically substantially round. The elongation (A₁₀) of the steel wire rod used in the method according to the invention is typically 25 - 35%. Typically, the tensile strength Rₘ of the steel wire rod is 370 - 420 N/mm² and the yield strength R_{P0,20} is 320 - 370 N/mm².

A typical steel wire mesh, preferably a steel wire mesh for mining applications, is manufactured from substantially smooth-surface steel wire, i.e. from further processed rod wire.

In one preferred embodiment of the invention steel wire rod having a diameter of 5.5 mm or 6 mm is used as a material of the steel wire mesh for mining applications. Since the method of the invention does not substantially affect to the diameter of the wire, the steel wire mesh according to the invention is thus manufactured from the steel wire, the diameter of which is about 5.5 mm or 6 mm. The diameter of the wire affects the mesh size of the mesh to be manufactured, so that the desired strength and weight of the mesh is achieved. The diameter of the wire and the mesh size of the mesh to be manufactured from it is chosen according to the purpose of use.

The mesh-like structure is formed of cut processed parts of the steel wire rod, i.e. steel wire, and the parts of the wire rod overlapping in the structure are welded together at locations, where the parts intersect.

### Detailed description of the invention

In the following the invention will be described in more detail with reference to the appended Figure 1, which illustrates the method of the invention.

In the method of Figure 1 steel wire rod 2 used as a raw material of the mesh-like structure 1 is guided to a further processing stage 10, in which the wire rod 2 is guided either through at least one drawing stone or rolling unit so that the roll scale is removed from the surface of the wire rod. After the further processing stage 10 the processed wire rod 3 can be recoiled before the processed wire rod 3, i.e. the steel wire, is further guided to the next stage 20, in which the steel wire 3 is straightened and cut into parts 4, 4' having a desired length. The straightening of the wire means smoothing out the wire, so that substantially straight elongated parts 4, 4' can be cut from the wire.

A mesh-like structure, preferably a steel wire mesh for mining applications 1, is formed by welding from the parts 4, 4' cut from the steel wire 3. The mesh structure 1 is welded at the intersections, where the parts 4, 4' arranged in different directions relative to each other overlap.

In the following is described an example of a steel wire mesh for mining applications manufactured by the method according to the invention.

### Example (not according to claim 1)

The manufacture of the mesh employs a wire rod made of steel, which wire rod has
- an average diameter of 5.5 mm
- an elongation A₁₀ = 25 - 30%
- a tensile strength Rₘ = 370 - 420 N/mm²
- a yield strength R_{P0,20} = 320 - 370 N/mm²

The wire rod is drawn through a drawing stone, which has an aperture of 5.5 mm, or through a rolling unit, which is set for the diameter of 5.5 mm, so that the roll scale can be removed from the surface of the wire rod (so-called calibration stretch). The average diameter of the processed wire rod is not more than 1.5% smaller than the diameter of the unprocessed wire rod.

After the calibration stretch the smooth surface steel wire is straightened and cut into parts having a desired length. The mesh-like structure having a desired size is welded from the cut parts. The size of the steel wire mesh is for example 2270 mm x 2530 mm, and the mesh size of the mesh is 75 mm x 75 mm, wherein the desired strength and shapability properties of the mesh are achieved.

The invention is not intended to be limited to the above-presented exemplary embodiments, but the intention is to apply the invention widely within the scope defined by the claims defined below.

## Claims

1. Method for manufacturing a steel wire mesh (1) for mining applications, from steel wire rod (2), in which method
- steel wire rod (2) having a specific diameter is guided to a further processing stage (10) where roll scale and other possible impurities are removed from the surface of the steel wire rod,
- the processed steel wire rod (3) is straightened and cut into parts having a desired length,
- the desired steel wire mesh (1) is welded from the cut steel wire parts (4, 4'),
wherein the method is free from heat treatment stages,
**characterized in that**
- the average diameter of the steel wire rod (2) remains substantially the same in the further processing stage, and the diameter of the steel wire rod is formed more circular, the change of the average diameter of the steel wire rod being 0.01-0.75%,
- the steel wire rod is only guided through the further processing stage and the straightening stage before forming the actual mesh structure by welding.

2. Method according to claim 1, **characterized in that** the further processing (10) of the steel wire rod is performed by guiding the steel wire rod (2) through at least one drawing stone, the drawing stone aperture having a diameter, which is substantially the same as the diameter of the steel wire rod.

3. Method according to claim 1, **characterized in that** the further processing (10) is performed by guiding the steel wire rod (2) through one or more rolling units.

4. Method according to any of the preceding claims, **characterized in that** the steel wire rod is typically guided directly from the further processing stage to a straightening stage, only through an optional intermediate coiling, but without any intermediate steps which would affect the strength properties of the steel wire.

5. Method according to any of the preceding claims, **characterized in that** the propagation speed of the steel wire rod in the further processing stage is substantially the same as the maximum speed of a wire coiling unit used in the further processing.

6. Method according to any of the preceding claims, **characterized in that** the elongation (A₁₀) of the steel wire rod is 25 - 35% and its tensile strength Rₘ is 370 - 420 N/mm².

7. Method according to any of the preceding claims, **characterized in that** the average diameter of the steel wire rod (2) is about 5.5 mm or 6 mm.

## Patentansprüche

1. Verfahren zur Herstellung eines Stahldrahtgitters (1) aus Stahlwalzdraht (2) für den Bergbau, wobei bei dem Verfahren
- Stahlwalzdraht (2) mit einem spezifischen Durchmesser einer weiteren Verarbeitungsstufe (10) zugeführt wird, in der Walzzunder und andere mögliche Verunreinigungen von der Oberfläche des Stahlwalzdrahtes entfernt werden,
- der bearbeitete Stahlwalzdraht (3) geradegerichtet und in Teile mit einer gewünschten Länge geschnitten wird,
- das gewünschte Stahldrahtgitter (1) aus den geschnittenen Stahldrahtteilen (4, 4') geschweißt wird,
wobei das Verfahren frei von Wärmebehandlungsstufen ist,
**dadurch gekennzeichnet, dass**
- der mittlere Durchmesser des Stahlwalzdrahtes (2) in der weiteren Verarbeitungsstufe im Wesentlichen gleich bleibt und der Durchmesser des Stahlwalzdrahtes kreisförmiger geformt wird, wobei die Änderung des mittleren Durchmessers des Stahlwalzdrahtes 0,01-0,75% beträgt,
- Der Stahlwalzdraht nur durch die weitere Verarbeitungsstufe und die Gerade-Richtstufe geführt wird, bevor die eigentliche Gitterstruktur durch Schweißen geformt wird.

2. Verfahren nach Anspruch 1, **dadurch gekennzeichnet, dass** die weitere Verarbeitung (10) des Stahlwalzdrahtes durch Führen des Stahlwalzdrahtes (2) durch mindestens einen Ziehstein erfolgt, wobei die Ziehsteinöffnung einen Durchmesser, der im Wesentlichen gleich dem Durchmesser des Stahlwalzdrahtes, ist aufweist.

3. Verfahren nach Anspruch 1, **dadurch gekennzeichnet, dass** die weitere Verarbeitung (10) durch Führen des Stahlwalzdrahtes (2) durch eine oder mehrere Walzeinheiten erfolgt.

4. Verfahren nach einem der vorstehenden Ansprüche, **dadurch gekennzeichnet, dass** der Stahlwalzdraht typischerweise direkt von der weiteren Verarbeitungsstufe zu einem Gerade-Richtstufe geführt wird, nur durch eine optionale Zwischenwicklung, jedoch ohne Zwischenschritte, die die Festigkeitseigenschaften des Stahldrahtes beeinflussen würden.

5. Verfahren nach einem der vorstehenden Ansprüche, **dadurch gekennzeichnet, dass** die Weitergabegeschwindigkeit des Stahlwalzdrahtes in der weiteren Verarbeitungsstufe im Wesentlichen gleich der maximalen Geschwindigkeit einer bei der weiteren Verarbeitung verwendeten Drahtwickeleinheit ist.

6. Verfahren nach einem der vorstehenden Ansprüche, **dadurch gekennzeichnet, dass** die Dehnung (A₁₀) des Stahlwalzdrahtes 25 - 35% und seine Zugfestigkeit Rₘ 370 - 420 N/mm² beträgt.

7. Verfahren nach einem der vorstehenden Ansprüche, **dadurch gekennzeichnet, dass** der mittlere Durchmesser des Stahlwalzdrahtes (2) etwa 5,5 mm oder 6 mm beträgt.

## Revendications

1. Procédé de fabrication d'un treillis en fil d'acier (1) pour des applications d'exploitation minière, à partir d'une tige en fil d'acier (2), procédé dans lequel
- une tige en fil d'acier (2) ayant un diamètre spécifique est guidée vers un étage de traitement supplémentaire (10) où des calamines de laminage et autres impuretés éventuelles sont éliminées de la surface de la tige en fil d'acier,
- la tige en fil d'acier (3) traitée est redressée et coupée en parties ayant une longueur souhaitée,
- le treillis en fil d'acier (1) souhaité est soudé à partir des parties en fil d'acier coupé (4, 4'),
dans lequel le procédé est exempt d'étages de traitement thermique, **caractérisé en ce que**
- le diamètre moyen de la tige en fil d'acier (2) reste sensiblement le même dans l'étage de traitement supplémentaire, et le diamètre de la tige en fil d'acier est formé davantage circulaire, le changement du diamètre moyen de la tige en fil d'acier étant de 0,01 à 0,75 %,
- la tige en fil d'acier est guidée uniquement à travers l'étage de traitement supplémentaire et l'étage de redressement avant de former la structure de treillis réelle par soudage.

2. Procédé selon la revendication 1, **caractérisé en ce que** le traitement supplémentaire (10) de la tige en fil d'acier est réalisé en guidant la tige en fil d'acier (2) à travers au moins une pierre d'étirage, l'ouverture de pierre d'étirage ayant un diamètre, qui est sensiblement le même que le diamètre de la tige en fil d'acier.

3. Procédé selon la revendication 1, **caractérisé en ce que** le traitement supplémentaire (10) est réalisé en guidant la tige en fil d'acier (2) à travers une ou plusieurs unités de laminage.

4. Procédé selon l'une quelconque des revendications précédentes, **caractérisé en ce que** la tige en fil d'acier est typiquement guidée directement depuis l'étage de traitement supplémentaire jusqu'à un étage de redressement, uniquement à travers un bobinage intermédiaire facultatif, mais sans étapes intermédiaires qui affecteraient les propriétés de résistance mécanique du fil d'acier.

5. Procédé selon l'une quelconque des revendications précédentes, **caractérisé en ce que** la vitesse de propagation de la tige en fil d'acier dans l'étage de traitement supplémentaire est sensiblement la même que la vitesse maximale d'une unité de bobinage de fil utilisée dans le traitement supplémentaire.

6. Procédé selon l'une quelconque des revendications précédentes, **caractérisé en ce que** l'allongement (A₁₀) de la tige en fil d'acier (2) est de 25 à 35 % et que sa résistance à la traction Rₘ est de 370 à 420 N/mm².

7. Procédé selon l'une quelconque des revendications précédentes, **caractérisé en ce que** le diamètre moyen de la tige en fil d'acier (2) est d'environ 5,5 mm ou 6 mm.
